

## UNITED STATES PATENT OFFICE

2,159,982

LEAD ALLOY AND METHOD OF PREPARING  
THE SAME

Nettie M. Hurd Bullock, Orlando, Fla.

No Drawing. Application January 5, 1937,  
Serial No. 119,081

7 Claims. (Cl. 75—166)

This application refers to metals and more particularly to an alloy composed mostly of treated lead, and is a continuation in part of my prior application, Serial No. 84,562, filed June 10, 1936.

5 Certain metals are unsuited for many uses, due to their susceptibility to corrosion by acids, their oxidation, tarnish, and general disintegration under weather conditions. Many metals which are to be subjected to the elements or to contact 10 with liquids which corrode them ordinarily are previously treated by dipping, or electrolytic processes to coat them with another product, which is less susceptible to the substances in connection with which said metals are to be used. One of the more familiar processes to be used in coating such metals is galvanizing, although there are a number of others. These 15 various processes are objectionable, inasmuch as a coating is usually brittle and is, to a great extent, porous. Wherever porosity occurs, the base metal is subjected to the substance from which protection is desired, and its life is thus shortened and its usefulness impaired.

Moreover, there are functional difficulties in 20 applying coatings of various types as a great many of these coatings require a high temperature which has a deteriorating effect on the metal to be coated; as, for instance, in the case of steel, where the temper of the steel is injured 25 by subjection to high temperatures. Moreover, many of these coatings are crystalline in their nature, and as a result, will not stand up under friction or pressure. It is often desirable to make certain articles out of lead but due to the nature 30 of the product and its porosity as well as its tendency to darken, this product is objectionable.

An object of this invention is to produce a metal and a method for the production of such a metal, which will overcome many of the disadvantages inherent in known coatings. A further object is to produce a metal which may be used in place of lead, in which the porosity of lead is greatly reduced and which will be free from corrosion or tarnish, thus maintaining its brilliance.

45 A still further object is to provide a lead alloy in which the crystalline structure is not discernible, and which will be very fluid when molten so as to be easily applied as a coating for metals, and when so applied, will fill pores and fasten 50 itself to said metal, in such a way as to make a permanent and lasting coat. A still further object is to provide a coating which may be applied to all metals at low temperatures and may be thus used without destroying or injuring the 55 metal to which it is applied.

Another object is to provide a metal from which many if not all of the poisonous characteristics of lead have been removed and which, not being subject to oxidation, is safe for use in children's toys and in similar trinkets.

A still further object is to provide a method of preparing an alloy which may, by the addition or omission of minor steps in process, be suited for a variety of purposes.

With these and other objects which will become apparent as the description proceeds, my invention consists in the product and method of producing the same hereinafter described. It will be appreciated that both the product and the metal may and can be varied in slight detail to fit the product to particular uses and to give it certain desired characteristics and qualities.

In preparing my product, I mix a quantity of lead, preferably cut in small pieces, nitric acid, sulphuric acid, and clay, or fuller's earth, under agitation. Of the entire mass by weight, the ingredients are mixed in the following percentages or proportions:

|                                                  | Per cent |    |
|--------------------------------------------------|----------|----|
| Lead (Pb)                                        | 82.6     | 25 |
| Nitric acid (HNO <sub>3</sub> )                  | 6.2      |    |
| Sulphuric acid (H <sub>2</sub> SO <sub>4</sub> ) | 3.1      |    |
| Clay, fuller's earth                             | 8.1      |    |
|                                                  | 100.00   | 30 |

This mass is allowed to work while being constantly agitated, until the chemical re-action is complete. This takes about thirty (30) minutes.

The entire mass is then heated, while being agitated, at about 700° F. until a residue forms at the top as a scum. This scum apparently consists of various impurities, contained in normal lead and this process and the following steps remove such impurities and take with them their disadvantages. This scum is then skimmed off or 35 the molten metal tapped off from the bottom. The molten metal represents by weight about 66.67% of the weight of the original ingredients; 1/3 of the weight of the ingredients either evaporating or being left in the scum that forms at 40 the top of the cauldron or retort.

Further refinement of the metal thus produced may be accomplished by the use of one or more of the following steps and the metal is kept at 700° F., still under agitation. To about .91.427 parts 45 of the metal, about .054 part sodium chloride (NaCl) and the mass agitated until a scum forms, which scum is then removed, and to the remaining metal, about .67 part sodium silicate (Na<sub>2</sub>SiO<sub>3</sub>) are added. Again scum forms and is removed 50

or the molten metal tapped off. About .107 part oxalic acid ( $H_2C_2O_4$ ) is then added, and the process repeated, still under agitation. Bismuth to the extent of about .861 part and 6.880 parts 5 of tin are then added to the molten mass and agitated until thoroughly mixed.

The molten mass may be cast into pigs or if to be used for dipping, passed into dipping tanks. Further refinement of the metal may be produced by adding copper acetate, sodium carbonate, potassium hydroxide or acetic acid, in amounts varying from  $\frac{1}{2}$  to 2 parts, as compared to the metal. The use of these products tends to further purify the metal and to better suit it for 10 varying purposes. The use of copper acetate, for instance, tends to make the metal whiter, stronger and to make it considerably harder. When sodium carbonate or potassium hydroxide is used, the metal is likewise made whiter and is more 15 suitable for decorative purposes, such as castings and novelties.

The metal thus produced is one in which the crystalline structure is not discernible and the porosity which exists in lead is, to a great 20 extent, removed.

It may be applied to other metals by dipping or other suitable means at temperatures as low as 665° F. and it has been found that, when so applied to steel and other metals, it cannot be 25 effectively removed by friction, heat or otherwise. Moreover the metal is flexible and has a brilliant appearance, being almost white in color. It will not tarnish when subjected to the elements and resists acids, alkalies, salt water, and 30 other substances which normally produce corrosion or oxidation.

It may be applied as a coating for all sorts of metals and is so fluid when molten that nuts and bolts and similar apparatus may be coated 35 without effecting their fit. Obviously, while I have set forth many uses such as coatings, the manufacture of lead toys, lining for tanks, etc., many other uses are apparent such as plates for storage batteries, and in other uses where lead 40 is desired. In the case of storage batteries, the metal is not seriously affected by sulphuric acid fumes, and plates made of this metal are much 45 more durable.

While in this specification, I have discussed my 50 process with reference to lead, it is equally suited to other metals and when applied to aluminum and copper, produces an alloy which strongly resists corrosion. While I have indicated the series 55 of steps which produces the finished product, the latter steps may be eliminated and at the same time, the method will produce an alloy of very fine structure and high degree of purity.

I claim:

1. A process of preparing an alloy which consists in mixing, under agitation a metal such as lead with approximately 6% by volume of nitric acid, approximately 3% by volume of sulphuric acid, and approximately 8% by volume of clay until the chemical reaction has substantially 60 ceased, then heating the mixture until thoroughly molten under agitation and until a scum forms, and then separating the scum from the metal.

2. A process of preparing an alloy which consists in mixing, under agitation, a metal such as lead with approximately 6% by volume of nitric acid, approximately 3% by volume of sulphuric acid and approximately 8% by volume of clay until the chemical reaction has substantially 70 ceased, then heating the mixture until thorough-

ly molten under agitation and until a scum forms, and then separating the scum from the metal, adding under agitation approximately  $\frac{1}{20}$  of 1% by volume of sodium chloride, removing the resultant scum and adding approximately two-thirds of 1% by volume of sodium silicate, under agitation and again removing the resultant scum. 75

3. A process of preparing an alloy which consists in mixing, under agitation, a metal such as lead with approximately 6% by volume of nitric acid, approximately 3% by volume of sulphuric acid, and approximately 8% by volume of clay until the chemical reaction has substantially 10 ceased, then heating the mixture until thoroughly molten under agitation and until a scum forms, and then separating the scum from the metal, adding approximately one-quarter of 1% by volume of oxalic acid and removing the resultant scum.

4. A process of preparing an alloy which consists in mixing, under agitation, a metal such as lead with approximately 6% by volume of nitric acid, approximately 3% by volume of sulphuric acid, and approximately 8% by volume of clay until the chemical reaction has substantially 15 ceased, then heating the mixture until thoroughly molten under agitation and until a scum forms, and then separating the scum from the metal, adding thereto approximately 1% by volume of bismuth and approximately 8% by volume of tin. 20

5. A method of preparing an alloy which consists in treating approximately 86 parts of a metal such as lead with 6 parts of nitric acid and approximately 3 parts of sulphuric acid in the presence of about 8 parts of fuller's earth, agitating the same until the chemical reaction is substantially diminished, then heating the mass 25 at about 700° F. until a scum forms, and removing said scum.

6. A method of preparing an alloy which consists in mixing under agitation a metal such as lead with approximately 6% by volume of nitric acid and approximately 3% by volume of sulphuric acid and approximately 8% by volume of clay, until the chemical reaction has substantially 30 ceased and heating the mixture until thoroughly molten and until a scum forms, separating the scum from the metal and adding under agitation approximately  $\frac{1}{20}$  by volume of sodium chloride, removing the resultant scum, and 35 then adding approximately two-thirds of 1% by volume of sodium silicate, again removing the resulting scum, treating the remaining metal with approximately one-quarter of 1% by volume of oxalic acid and again removing the scum, and then adding thereto approximately 1% of bismuth and 8% of tin. 40

7. A process of preparing an alloy which consists in mixing under agitation a metal such as lead with approximately 6% by volume of nitric acid, 3% by volume of sulphuric acid, and approximately 8% by volume of fuller's earth until the chemical reaction has substantially ceased, then heating the mixture under agitation until thoroughly molten and until a scum forms, removing the scum from the metal and adding  $\frac{1}{20}$  of 1% by volume of sodium chloride, again agitating the mixture and removing the scum, then adding approximately two-thirds of 1% of sodium silicate, agitating the metal, removing the resulting 50 scum, then adding approximately one-quarter of 1% oxalic acid, reagitating, and again removing the resulting scum and adding thereto approximately 1% of bismuth and 8% of tin. 55

NETTIE M. HURD BULLOCK. 75